

C. F. CARRIER, JR.

METHOD OF DETINNING.

APPLICATION FILED AUG. 5, 1911. RENEWED AUG. 7, 1920.

1,358,136.

Patented Nov. 9, 1920.

2 SHEETS—SHEET 1.



WITNESSES:

Minerva Lobel  
M. A. Bell

INVENTOR:

Courtland F. Carrier Jr.,

BY

Flann, David & Oldsborough,  
ATTORNEYS

C. F. CARRIER, JR.

METHOD OF DETINNING.

APPLICATION FILED AUG. 5, 1911. RENEWED AUG. 7, 1920.

1,358,136.

Patented Nov. 9, 1920.

2-SHEETS—SHEET 2.



# UNITED STATES PATENT OFFICE.

COURTLAND F. CARRIER, JR., OF CHARLESTON, WEST VIRGINIA, ASSIGNOR TO THE VULCAN DETINNING COMPANY, OF SEWAREN, NEW JERSEY, A CORPORATION OF NEW JERSEY.

## METHOD OF DETINNING.

1,358,136.

Specification of Letters Patent.

Patented Nov. 9, 1920.

Application filed August 5, 1911, Serial No. 642,470. Renewed August 7, 1920. Serial No. 402,030.

To all whom it may concern:

Be it known that I, COURTLAND F. CARRIER, Jr., a citizen of the United States, and resident of Charleston, county of Kanawha, State of West Virginia, have invented certain new and useful Improvements in Methods of Detinning; and I do hereby declare the following to be a full, clear, and exact description of the invention, such as will enable others skilled in the art to which it appertains to make and use the same.

My invention relates to what is known as chlorin detinning, an art which is founded upon the well known principle that dry chlorin gas has a strong affinity for tin without affecting iron. Tin scrap when subjected to dry chlorin may, by the proper application of this principle, have its tin surface converted into stannic chlorid, leaving the iron substantially free from tin and unaffected by the chlorin or stannic chlorid. My invention has for its object to apply this well known principle on a commercial scale in such a manner as to obtain great efficiency of action and purity of product.

Heretofore, in the carrying out of chlorin detinning on a commercial scale, many difficulties were encountered as the result of attempts to regulate the temperature in the apparatus in which the detinning operation is carried on; and also resulting from the pressures created in said apparatus, and from the manipulation of the materials. It is the object of the present invention to devise a process which dispenses entirely with those things heretofore recognized as creating defects, and to devise a process which shall be continuous from start to finish, which shall operate practically automatically, and in which no regulation of temperature whatsoever is necessary and no pressures are created, and in which all of the elements of the process do their normal work without requiring any positive manipulative control and without the creation of any unusual circumstances or conditions.

The apparatus in which my process may be advantageously carried out is illustrated in the drawings, in which—

Figure 1 illustrates in front elevation apparatus suitable for the practice of the invention;

Fig. 2 represents a top plan view thereof;

Fig. 3 represents a rear elevation;

Fig. 4 represents a side elevation; and

Fig. 5 represents a partial vertical sec-

tion, on a somewhat larger scale, of one of the units of the apparatus.

In the drawings, A<sup>1</sup>, A<sup>2</sup>, A<sup>3</sup>, A<sup>4</sup>, A<sup>5</sup> and A<sup>6</sup> represent a series of six (6) cylinders, 60 each provided with tight-fitting lids B, having a lug and ring for convenience in handling. Each cylinder is conveniently fitted with a test-pipe b for drawing samples of gases. 65

The series connection is made by joining the opposite ends of adjacent cylinders by pipes D, and a closed series is formed by joining the cylinder A<sup>6</sup> with the cylinder A<sup>1</sup> by the pipe E. The pipes D and E are 70 provided, respectively, with hand-valves d and e. The cylinders are also connected in parallel by means of the chlorin supply-pipe F; the air line G; the exhaust line H; the by-pass line I; the double gas line J; 75 and the stannic chlorid line K. All of these lines are connected to each of the cylinders by means of branch pipes in which are located the hand-valves f, g, h, i, j, k, respectively. 80

The gas line J has a connection to the top of each cylinder and at both ends of the cylinder, as shown, and a blower L is interposed in the line J at some convenient point between the two sets of connections; so that, 85 by this arrangement, gas can be pumped from any one of the cylinders and blown into any other cylinder at will. So also, the air may be supplied to any individual cylinder or cylinders by the air line G, 90 connected with any suitable source of air supply. Furthermore, any of the cylinders may be supplied with chlorin from the line F, and connections can be made from any of the cylinders with the lines H, I, and K, respectively, at will. As shown in the drawings, the chlorin line F, the by-pass line I, and the stannic chlorid line K are most conveniently connected to the bottom of each of the cylinders at one end thereof, and the air 100 line G and exhaust line H to the top of the cylinders at the other end.

In the drawings, the cylinders are shown as in a horizontal position, which is preferable, especially, where they are of large 105 size, for a number of reasons, particularly because when supported in the horizontal position, they can sustain to better advantage their own weight and the weight of their contents of tin scrap and the containers therefor. It will, of course, be understood that nevertheless, in many in-

stances, it will be found convenient to arrange the cylinders either at an incline or even in the vertical position, according to the requirements or convenience of local 5 conditions. So also, the pipes D and E may either connect the tops of the cylinders, as shown, or they may connect the cylinders in any other suitable way, as, for instance, by joining the top of one cylinder 10 with the bottom of the next in the series.

The drawing illustrates a convenient number of cylinders but the number may obviously be varied; for instance, a lesser number may be employed, although I do not recommend the employment of less than four. It is also to be understood that the cylinders and various parts may of any convenient form and that they should be constructed of a material which will resist the 15 action of the substances involved in the practice of the process.

The tin scrap to be treated is placed in suitable baskets or receptacles such as perforated iron, or screens. A sufficient number of these baskets is provided and they are of a size to fit the cylinders and to substantially fill the same. A convenient number is also kept in reserve at all times. For the purpose of illustration, I have shown in 20 Fig. 5, one of the baskets partially filled. The scrap which fills these baskets is ordinarily cleaned by any conventional method and dried before it is placed in the cylinders and the baskets of dry scrap are 25 placed in the cylinders without giving them an opportunity to condense moisture from the air. The cylinders are closed when they are filled with this dry scrap and the lids B are fastened air tight. The valves in the 30 pipe system are so arranged that a current of chlorin gas will be admitted to the cylinder A<sup>1</sup> and such portions of this chlorin as are not consumed in the reaction in that cylinder will pass on into the cylinder A<sup>2</sup>. 35 and so on through the various cylinders. At the same time that the chlorin is admitted, the blower L is set in motion, thereby supplying the cylinder A<sup>1</sup> with a large volume of dry air which carries the chlorin 40 through the cylinder A<sup>1</sup> in a diluted condition. A large part of the diluted chlorin will react with the tin on the scrap and form stannic chlorid which being liquid, trickles to the bottom of the cylinder and 45 is withdrawn through the line K. The valve j on cylinder A<sup>5</sup> being open, the air that may be contained in the cylinders originally will be forced through the line J into the cylinder A<sup>1</sup>. The cylinder A<sup>5</sup>, in addition to having this connection to the line J, also connects with the cylinder A<sup>6</sup>, and the cylinder A<sup>6</sup> is open only to the exhaust line H. The connection through E between cylinders A<sup>1</sup> and A<sup>6</sup> is closed and the gases 55 which escape from A<sup>6</sup> pass out of the sys-

tem where they may be subjected to further treatment for the recovery of any valuable constituents. The volume of air supplied through line J is exceedingly large compared with the volume of chlorin so that 70 the chlorin in the system at that period of the operation is throughout in a state of great dilution.

When the detinning operation is started originally, it will be noted that the scrap 75 has its full coating of tin in each of the cylinders. The chlorin being very dilute attacks this coating of tin and converts it into stannic chlorid (SnCl<sub>4</sub>). As the reaction proceeds, a point will finally be reached 80 where the dilute chlorin which has been admitted in the cylinder A<sup>1</sup> will no longer react with any of the tin contents of the scrap and when that point has been reached, the connection between the line J and cylinder A<sup>1</sup> is closed, and the connection between J and the cylinder A<sup>2</sup> is opened. The supply of strong chlorin to A<sup>2</sup> is continued. The effect of this is that the cylinder A<sup>1</sup> will be filled with chlorin of maximum strength which, following immediately upon a condition of great dilution of chlorin removes from the scrap in the cylinder A<sup>1</sup> the remaining portions of tin. The surplus of concentrated chlorin passes 95 through the line D into the cylinder A<sup>2</sup> where it is again diluted as it had been in the cylinder A<sup>1</sup> by a large volume of air from the pipe J.

Next, the valve d in the pipe D which 100 connects cylinders A<sup>1</sup> and A<sup>2</sup> is closed. The chlorin is shut off from cylinder A<sup>1</sup> and admitted into cylinder A<sup>2</sup>. In order to clear cylinder A<sup>1</sup> of chlorin, the by-pass connections are made between cylinders A<sup>1</sup> and A<sup>3</sup> 105 and air is admitted through the air line G into the cylinder A<sup>1</sup>. After the residual fumes have been blown out, the detinned material is removed from cylinder A<sup>1</sup>, and it is then refilled with fresh scrap. The 110 complete removal of the fumes is determined by testing a sample of gases drawn from the test pipe b.

The connections between A<sup>6</sup> and A<sup>1</sup>, through pipe E, between A<sup>1</sup> and the exhaust line H, and between A<sup>6</sup> and the blower-intake branch of line J are opened and the connection which had theretofore existed between A<sup>5</sup> and said blower-intake branch of the line J is closed. In this way, cylinder A<sup>2</sup> has become the first of the series and cylinder A<sup>1</sup> the last of the series. By the time these connections have all been made, the diluted chlorin in cylinder A<sup>2</sup> has finished its work and that cylinder is ready for 125 the strong chlorin treatment which proceeds as before described in connection with cylinder A<sup>1</sup>, and so on throughout the system.

The chlorin which is employed in this process should be dry when used. It may 130

be derived from any convenient source. If produced from a commercial chlorin generating battery system the chlorin will contain a fairly large amount of air. On the other hand, practically pure chlorin may be supplied from liquid chlorin containers or any other source. The air that is used should also be thoroughly dry. The air that is used for clearing the cylinders of their remaining contents of chlorin gas is preferably dry, dehydrated, warm air. Such chlorin as escapes from cylinder A<sup>1</sup> into cylinder A<sup>2</sup> is in a dilute condition even after all reaction in the cylinder A<sup>1</sup> has ceased and as this diluted chlorin passes through the series, it displaces any air or gas that may be contained in all of the other cylinders and pushes it forward. There is an increasing quantity of tin on the scrap in each of the cylinders in the series, the last cylinder being obviously subjected to a dilute chlorin treatment in presence of such an excess of tin that practically none of the chlorin can pass out of the system without entering into the reaction with the tin.

It will readily be seen that, in the process described, the detinning operation is conducted uniformly and continuously, such conditions being favorable to uniformity of result. The main operative advantage of the process is to be found, however, in the separation of the operations into separate successive stages each of which is peculiarly adapted to the work it is to accomplish. Thus it will be seen that one cylinder will be in the absorption stage, three will be in the detinning stage, and one in the finishing stage, and the sixth cut out for fume removal and refilling. It will also be seen that the operation is so conducted that the fresh scrap is first treated with extremely diluted chlorin produced as residual gas from the earlier stages of the process. This starts the detinning and as there is a large excess of tin present only a minimum amount of chlorin if any, can escape. In the next stage, a dilute chlorin formed by the impoverishment of the gaseous mixture before reaching that stage will have a slightly stronger effect but still within the limits of very dilute chlorin. In the next stage, detinning is completed so far as dilute chlorin can accomplish it and in the final stage by a sudden injection of concentrated chlorin following the dilute chlorin treatment the remaining portions of the tin are removed.

The efficiency of such a process is greatly influenced by the state of rest or the state of motion of the gases during the several stages of the operation. The absorption stage is more complete and efficient if the dilute chlorin is in a state of comparative rest or quiet. Under such conditions owing to the greater density of the chlorin the gas

tends to stratify. As the consumption of the chlorin progresses the gaseous mixture will become less dense than before and there will be a constant tendency to stratification in the vessel, the less dense portions of the gaseous mixtures rising progressively above those portions which contain larger percentages of chlorin. If, therefore, the gases in the absorption stage be kept as quiescent as possible the gases escaping from the vessel will contain minimum percentages of chlorin. For this reason it is preferred to keep the gases in as quiescent a state as possible during the absorption. The detinning stage has considerably different requirements. The reaction between chlorin and tin generates heat and if this is localized the iron as well as the tin will be consumed. This localization of heat is possible when the gases are in a quiescent state, but if the gases are diluted and the heat is diffused no such localization of heat takes place. By keeping the gases in a violent state of circulation during the detinning stage, the percentage of the chlorin in the gas is substantially the same in all parts of the apparatus, hence, the reaction takes place at all points simultaneously and the heat is uniform throughout the apparatus.

It is also to be noted that while a chance inequality of temperature between two points in the system would be quickly balanced by the circulating gases, any serious inequality of temperature cannot arise, even temporarily, as is more fully explained below. Furthermore, while the bulk of the detinning is best accomplished by means of a rapidly circulating current of dilute chlorin gas, it has also been observed that the dilute gas has not the reactive power of concentrated chlorin and that that portion of the tin which is in immediate contact with the iron and which forms therewith a tin-iron alloy is not attacked by dilute chlorin but is attacked by strong chlorin. The finishing stage of the operation, involving the employment of concentrated chlorin is, therefore, necessary in order to obtain the maximum detinning effect; and, inasmuch as full penetration of the mass of the tin scrap is not so readily attained during the circulating stage wherein dilute chlorin is employed, the quiescent stage is made available for a complete penetration of the mass by displacement with the concentrated chlorin.

The exigencies of the finishing stage are somewhat analogous to those of the absorption stage. The stratification principle is therefore, made use of in this case. The difference in density between air and dilute chlorin is not sufficient to displace the air from the interstices of the scrap while the gases are in motion. By maintaining the gases through the finishing stage in a substantially quiescent state, however, the less

dense gases are displaced and the heavy, concentrated chlorin readily penetrates the scrap. In this manner, the gases and the strong chlorin are brought into contact with 5 all portions of the tin. It is also much easier to increase the concentration of the chlorin to full strength by displacing in a quiet state than it would be to accomplish that result by a continual enrichment during circulation. It is also important that 10 the distances which the gases traverse shall be sufficiently great to allow the necessary time to elapse for the maximum amount of detinning by dilute chlorin, so that the 15 change from dilute to strong chlorin will be a sudden and not a gradual one.

By the use of this process all temperature regulation is avoided. No regulation whatsoever is necessary. The greater portion of 20 the tin being removed by dilute chlorin, is readily removed at temperatures far below those at which chlorin and iron unite, so that by the time the concentrated chlorin treatment is reached, there is not sufficient 25 tin on the scrap to produce abnormally high temperatures. This is the result of treating the fresh scrap first with the residual gases from the other parts of the process, then with diluted chlorin of slightly increasing 30 concentration until nearly all of the tin is removed, and finally, removing the maximum amount of the remaining tin in a finishing stage by means of very concentrated chlorin. The proportion of neutral 35 gases in the dilute chlorin is so great that the heat of the reaction is carried away by the depleted gases which are displaced by the fresh supply of highly diluted chlorin, for which reason it is impossible to over- 40 heat the scrap, and consequently no temperature control whatever is needed.

The essence of this invention, therefore, consists in a detinning process in which, once in working order, the fresh scrap is 45 treated under conditions of chlorin dilution, the last period of which is a chlorin in a high state of dilution; second, in following this dilute chlorin treatment, immediately with a concentrated chlorin treatment; and 50 third, in creating in the process the appropriate conditions of rest and motion for the periods of absorption, detinning and finishing. These three features which are simultaneously present in the process as above described, result in a chlorin detinning process 55 which, as described, is practically continuous and free from all complications such as temperature regulation or graduations of pressure or any special treatments. The entire process proceeds normally and without 60 the creation of any unusual conditions.

Having thus described my invention, what I claim is:

1. The method of detinning tin-scrap, 65 which consists in treating the scrap in separate portions, in separate, successive stages,

first with dilute anhydrous chlorin, until the major portion of the tin is removed, the dilution of the chlorin thus employed being so extreme that reaction with the iron of the scrap under the conditions prevailing is 70 impossible, and finishing the detinning with concentrated chlorin; substantially as described.

2. The method of detinning tin-scrap, 75 which consists in treating the scrap in separate portions, in separate, successive stages, first with dilute chlorin, until nearly all of the free tin is removed, the degree of dilution of the chlorin thus employed being such that under the prevailing conditions 80 reaction between the iron and the scrap is impossible, maintaining said degree of dilution practically uniform, and finishing the detinning with concentrated chlorin.

3. The method of detinning tin-scrap, 85 which consists in simultaneously treating separate portions of the scrap with dry chlorin of widely different degrees of concentration (*i. e.*, highly dilute and highly concentrated chlorin), in separate successive stages; substantially as described.

4. The method of detinning tin-scrap by means of chlorin which consists in treating separate portions of the scrap in separate, successive stages, with gaseous mixtures in 95 which the percentage of chlorin is abruptly increased after dilute mixtures have no further action; substantially as described.

5. The method of detinning tin-scrap by means of chlorin, which consists in removing the last portions of tin with an excess 100 of concentrated chlorin abruptly introduced after the major portion of tin has been removed by the action of dilute chlorin, and recovering the residues of chlorin by means of excess of tin; substantially as described.

6. The method of detinning tin-scrap by means of dry chlorin gas which consists in first utilizing the scrap to absorb residual chlorin, continuing the detinning with dilute 110 chlorin until the major portion of the tin is removed, and completing the detinning by the abrupt admission of an excess of concentrated chlorin; substantially as described.

7. The method of detinning tin-scrap, 115 which consists in carrying on the detinning operation by operating upon separate portions of the scrap in successive preliminary stages in the presence of dilute chlorin of gradually increasing concentration, and abruptly finishing the detinning in the presence of chlorin of a still higher degree of concentration; substantially as described.

8. The method of detinning tin-scrap by means of gaseous mixtures, which consists 125 in treating the scrap with a moving body of the gas, and then with a quiescent body thereof; substantially as described.

9. The method of detinning tin-scrap by means of gaseous mixtures, which consists 130

- in treating the scrap with a moving body of the gas, and then with a quiescent body thereof of a higher degree of concentration; substantially as described.
- 5 10. The method of detinning tin-scrap by means of gaseous mixtures, which consists in treating the scrap with the gas in varying states of rest and motion; substantially as described.
- 10 11. The method of detinning tin-scrap by means of gaseous mixtures, which consists in treating successive, separate portions of the scrap with the gas in varying states of rest and motion; substantially as described.
- 15 12. The method of detinning tin-scrap by means of gaseous mixtures, which consists in treating successive, separate portions of the scrap with the gas in varying states of rest and motion, the gas in the state of motion being diluted with gases previously used in the operation; substantially as described.
- 20 13. The method of detinning tin-scrap, which consists in treating the scrap with a circulating body of dilute chlorin, and finishing the detinning by treating the scrap with an excess of strong chlorin in a relatively quiescent state; substantially as described.
- 25 14. The method of detinning tin-scrap, which consists in treating the scrap with a circulating body of chlorin which has been diluted with the residue of gases previously used in the operation and then finishing the detinning with strong chlorin in a relatively quiescent state; substantially as described.
- 30 15. The method of detinning tin-scrap, which consists in treating the scrap with a body of rapidly circulating dilute chlorin to remove the bulk of the tin, removing the maximum amount of the remaining tin by treating the scrap with a large excess of strong chlorin in a relatively quiescent state, and recovering the maximum amount of the residual chlorin by treating the same with an excess of tin, while in a relatively quiescent state; substantially as described.
- 35 16. The method of detinning tin-scrap, which consists in treating the scrap with gaseous mixtures containing chlorin the gases being in a comparatively quiescent state when either the amount of free tin or chlorin approaches a minimum, and in such rapid state of circulation when considerable quantities of both tin and chlorin are present that the circulating chlorin gas mixture will be substantially uniform throughout; substantially as described.
- 40 17. The method of detinning tin-scrap, which consists in removing the greater portion of the tin with dry chlorin of such extreme dilution that under the prevailing conditions reaction with the iron of the scrap is impossible, and removing the maximum amount of the remaining tin with concentrated chlorin; substantially as described.
- 45 18. The method of detinning tin-scrap, which consists in first partially detinning a mass of scrap with chlorin in a state of dilution closely approaching an inert condition, and subsequently detinning such partially detinned mass to an extent sufficient to practically remove its remaining free tin contents by chlorin of such extreme dilution that under the prevailing conditions reaction with the iron of the scrap is impossible; substantially as described.
- 50 19. The method of detinning tin-scrap, which consists in first partially detinning a mass of scrap with chlorin in a state of dilution closely approaching an inactive condition, and subsequently detinning such partially detinned mass first with dilute chlorin of a strength less than that sufficient to practically remove its remaining free tin contents, and then completing the removal of said free tin, by means of chlorin of such extreme dilution that under the prevailing conditions reaction with the iron of the scrap is impossible; substantially as described.
- 55 20. The method of detinning tin-scrap, which consists in detinning a mass of scrap with dilute chlorin, depriving the partially spent gases of a further portion of the chlorin contents, then treating a mass of fresh scrap with said gases thus depleted, and then detinning said partially detinned fresh scrap with dilute chlorin of greater strength; substantially as described.
- 60 21. That improvement in the method of detinning tin-scrap by dilute chlorin, which consists in giving the fresh scrap a preliminary treatment with chlorin diluted to a state closely approximating an inert condition, employing a portion of the resultant gases as a diluent for chlorin and employing the chlorin thus diluted to remove further portions of tin from said partially detinned fresh scrap; substantially as described.
- 65 22. That improvement in the method of detinning tin-scrap with dilute chlorin, which consists in reducing the dilute chlorin employed as the active detinning agent to a state of extreme dilution, treating a mass of fresh scrap with such extremely diluted chlorin and employing the resultant impoverished gases as a diluent for the chlorin during some stage of its detinning activity before its condition of extreme dilution; substantially as described.
- 70 23. The method of detinning tin-scrap, which consists in establishing a series of separate charges to be treated; starting the operation in the first charge by the admission of chlorin gas diluted with air; decreasing the air dilution of the gas thus admitted as the detinning in said charge progresses; passing the gases from the first charge successively through the other charges of the series as the

detinning in the first charge proceeds; and finally by-passing the residual gases left after the completion of the detinning operation in the first charge into one of the charges utilizing dilute chlorin; substantially as described.

24. The method of detinning tin-scrap, which consists in establishing a series of separate charges to be treated; starting the operation in the first charge by the admission of chlorin gas diluted with air; decreasing the air dilution of the gas thus admitted as the detinning in said charge progresses; passing the gases from the first charge successively through the other charges of the series as the detinning in the first charge proceeds; finishing the detinning of the first charge by concentrated chlorin; and finally by-passing the residual gases left after the completion of the detinning operation in the first charge into one of the charges utilizing dilute chlorin; substantially as described.

25. The method of detinning tin-scrap, which consists in establishing a series of separate charges to be treated; starting the operation in the first charge by the admission of chlorin gas diluted with air; decreasing the air dilution of the gas thus admitted as the detinning in said charge progresses; passing the gases from the first charge successively through the other charges of the series as the detinning in the first charge proceeds; and finally by-passing, by means of a diluting current of warm, dry air, the residual gases left after the completion of the detinning operation in the first charge into one of the charges utilizing dilute chlorin; substantially as described.

26. The process of detinning which consists in circulating a mixture of chlorin gas and an inert gas (as air) through a succession of tanks containing tin scrap in varying stages of detinning, by introducing such inert gas to the tank containing the detinned scrap, and admitting fresh chlorin to a subsequent tank, the inert gas admixing therewith and being circulated serially through the successive tanks.

27. The process of detinning by circulating chlorin gas through a succession of tanks containing tin scrap in varying stages of detinning, which consists in introducing an inert gas (as air) into the tank containing detinned scrap, and circulating it thence through the series of tanks while introducing the chlorin to a subsequent tank in the series, whereby it forms a mixture with the inert gas, and circulates therewith until the chlorin is removed therefrom by combining with the tin.

28. The process of detinning by circulating chlorin gas through a succession of tanks containing tin scrap in varying stages of detinning, which consists in introducing an inert gas (as air) into the tank containing the detinned scrap, and introducing the strongest chlorin into a subsequent tank also containing detinned scrap, mixing said gases and circulating them through the subsequent tanks containing fresher charges of tin scrap until the chlorin is removed by combining with the tin.

29. The process of detinning by circulating chlorin gas through a succession of tanks containing tin scrap in varying stages of detinning, which consists in coupling said tanks in series except for one tank which is isolated from such series, opening said tank, removing the detinned scrap, recharging with fresh scrap and again closing it while the detinning operation is proceeding in the remaining tanks, then coupling the newly charged tank into the series and isolating therefrom the next succeeding tank for recharging, applying a suction each time at the outlet of the newly charged tank, admitting air to the tank longest charged with scrap, and admitting chlorin to a subsequent tank so that the chlorin and air may mix and be drawn together through the series of tanks.

In testimony whereof I affix my signature in presence of two witnesses.

COURTLAND F. CARRIER, Jr.

Witnesses:

MINERVA LOBEL,  
M. AGNUS BILL.